

## UNITED STATES PATENT OFFICE.

ARNOLD H. PETER, OF NEW YORK, N. Y.

## METHOD OF TREATING HIDES OR SKINS.

SPECIFICATION forming part of Letters Patent No. 727,832, dated May 12, 1903.

Application filed October 18, 1902. Serial No. 127,790. (No specimens.)

*To all whom it may concern:*

Be it known that I, ARNOLD H. PETER, a citizen of the Republic of Switzerland, residing in the city, county, and State of New York, have invented a new and useful Improvement in Methods of Treating Hides or Skins before Their Subsequent Immersion into a Tanning-Bath, and my process can be used with all kinds of hides and skins, and such hides or skins after treatment by my process may be tanned in either organic or metallic tanning-baths.

The object of my invention has been to dispense with and replace the costly, hazardous, and heretofore-considered indispensable processes known as "bating," "abating," "graining," "reducing," "degreasing," "drenching," and "puring." (See Davis, *The Manufacture of Leather.*)

By these operations above described I refer to all operations ordinarily performed on the hide or skin subsequent to the removal of the hair by "liming" and previous to the immersion of the hide or skin in the actual tanning-bath except washing and the mechanical operation of "fleshing" or "slating."

My invention consists in the discovery that hides and skins coming from the "lime" after undergoing the usual washing and the mechanical operation of fleshing can be put into suitable condition for immersion in the tanning liquor without resorting to bating, abating, graining, reducing, drenching, or puring, as is now commonly employed.

The elimination of the lime or alkali, the "letting out" or "opening up" of the hides or skins to overcome the shrinking effect of the lime, the smoothing and "letting down" of the grain, the starting of the "gelatinous" substances in the hide or skin and regulating its loss, the opening of the texture of the hide from its swollen gelatinous condition are all effectively accomplished by my treatment with a suitable acid and salt solution, applied as hereinafter specified. After treatment according to my process the acid and salt solution remaining in the hide can act upon it practically by what is known as "horsing" the hides. A perceptible change in the hide or skin will be noticed during the next twelve to forty-eight hours, and in this state the hides

or skins may be kept for a number of days without injury and ready for immersion in the actual tanning-bath. At the first glance at this state of the hides or skins they may appear somewhat similar to that presented by immersing them in an ordinary "pickle;" but the differences are very marked in the quality of the skin or hide before immersion in the tanning liquor, and I obtain this difference by the relative quantities of the salt and acid used in my process, which differ both in quantity and method of application from those heretofore used.

The following will serve as an illustration of a method of applying my process of treating the hides or skins with a suitable salt and acid solution for the purposes specified.

The hides or skins (after being taken from the lime and being unhaired, washed, and fleshed in the usual manner) are placed in an aqueous solution containing from one to five per cent. of chlorid of sodium and one-tenth of one per cent. of commercial muriatic acid, (HCL.) After a period of from one to two hours it will be found that almost all acid reaction has disappeared, and at this time another one-tenth of one per cent. of muriatic acid is to be added. After a further period of from one to two hours the acid reaction becomes very weak, and thus again one-tenth of one per cent. of muriatic acid is to be added. If the acid reaction should cease inside of two hours, now (the test to be made by the use of litmus paper or other indicator) another one-tenth of one per cent. of muriatic acid should be added; but if the acid reaction has not disappeared now within two hours no further acid should be added.

Some variations from the above working formula may be practiced without departing from the spirit of my invention. Thus, for instance, the hides or skins may be freed from superfluous liquor by mechanical means, such as "beating" or "working," or the superfluity may even be removed by washing. Again, the amounts of acid may be changed somewhat and instead of muriatic acid I can employ sulfuric acid ( $H_2SO_4$ ) or phosphoric acid ( $PO_4H_3$ ) or lactic acid, ( $C_3H_6O_3$ ). Still, again, the time of the intervals between adding each dose of the acid may vary and the temper-

ature at which the operations are performed may vary. In my tests I have found that the treatment can be carried on successfully at a degree of temperature as low 3° centigrade 5 and again as high as 40° centigrade, the degree of temperature being determined by the nature of the hides or skins and the effect on the grain, as different skins act differently under the same treatment. Thus the softer 10 natured skins, such as those of sheep and colts, require a lower temperature, and the harder skins, such as those of goats, permitting a higher temperature. The test, as is understood by practical tanners, is to be determined by the feel of the grain, whether it 15 is smooth or not and general appearances.

I do not confine myself to solutions specifically containing from one to five per cent. of salt, as I have successfully used solutions 20 containing up to twelve per cent. of salt and again down below one per cent. of salt.

My invention consists in the use of an acid and a salt solution for the treatment of hides or skins coming directly from the lime and 25 previous to immersion in the tanning liquor, in which the acid is used in such quantities and qualities only at the time that it is used that the acid will act to combine with the lime, but will not combine to any extent with 30 the substance of the hides. The affinity between the lime and the acid being greater than between the hide substance and the acid, my treatment renders it possible to remove the lime without causing the acid to combine 35 with the hide substance to any large extent, and thus leave the hide in its natural condition. The salt is to be used in such quantities only as to overcome the swelling action 40 of the acid on the skins or hides, and it is also used for the purpose of preventing a too-rapid action of the acid. The acid reaction depends or appears to depend on the electrolytical disassociation of the acid employed, and the presence of a salt of the acid reduces 45 or modifies this electrolytical disassociation, and thereby reduces the rapid action of the acid.

A further important part of my process consists in the discovery that the specific gravity (to be regulated by the amount of salt to be used in the solution) in which the hides or skins are to be immersed under my process before treatment with the tanning solution should be substantially the same as the specific gravity of the tanning-bath. By having these specific gravities coincide or nearly coincide I have discovered that there is little or no formation of strong currents of diffusion inside of the hides or skins after they 55 are removed from my salt and acid bath and immersed in the tanning-bath, and thus there is no undesirable effect produced upon the

texture of the hides, and consequently upon the ultimate texture of the leather produced therefrom.

I have discovered that the treatment of 65 hides and skins in the manner above described results in a fuller stronger leather of better grain and fiber and produced at a less expense than by the processes heretofore used 70 for similar purposes.

Having thus described my invention, what I claim is—

1. In tanning hides or skins, the process of 75 subjecting the hide or skin to the action of a solution of a salt into which relatively small quantities of an acid are introduced at intervals, substantially as and for the purpose set forth.

2. In tanning hides or skins, the process of 80 subjecting the hide or skin to the action of a solution of sodium chlorid into which relatively small quantities of acid are introduced at intervals, substantially as and for the purpose set forth.

3. In tanning hides or skins, the process of 85 subjecting the hides or skins to the action of an aqueous solution of sodium chlorid into which relatively small quantities of hydrochloric acid are introduced at intervals, sub- 90 stantially as and for the purpose set forth.

4. In tanning hides or skins, the process of 95 subjecting the hide or skin to the action of a solution of sodium chlorid into which acid is introduced at intervals, and subsequently subjecting the hides or skins to the action of a tanning-bath having substantially the same specific gravity as that of the salt and acid bath, substantially as and for the purpose set forth.

5. In tanning hides or skins, the process of 100 subjecting the hide or skin to the action of a solution of sodium chlorid into which relatively small quantities of acid at intervals are introduced, and subsequently subjecting the 105 hides or skins to the action of a tanning-bath having substantially the same specific gravity as that of the salt and acid bath, substan- tially as and for the purpose set forth.

6. In tanning hides or skins, the process of 110 subjecting the hide or skin to the action of an aqueous solution of sodium chlorid into which relatively small quantities of hydrochloric acid are introduced at intervals, and subse- 115 quently subjecting the hides or skins to the action of a tanning-bath having substantially the same specific gravity as that of the salt and acid bath, substantially as and for the purpose set forth.

ARNOLD H. PETER.

Witnesses:

MATTHEW W. WOOD,  
J. E. HINDON HYDE.